# EUROPEAN PATENT APPLICATION

(11) **EP 4 502 120 A1**
(43) Date of publication of application: **05.02.2025**
(21) Application number: 23779714.7
(22) Date of filing: 17.03.2023
(51) Int. Cl.: C10M 169/04, C10N 30/00, C10N 30/04, C10N 40/25, C10M 101/02, C10M 105/32, C10M 105/36, C10M 105/38, C10M 129/10, C10M 133/12, C10M 133/40

(54) **LUBRICANT COMPOSITION**

(30) Priority: 31.03.2022 JP 2022060211
(71) Applicant: Idemitsu Kosan Co.,Ltd., Tokyo 100-8321 (JP)
(72) Inventor: OKI, Hiroshi, Tokyo 100-8321 (JP); YAMASHITA, Jun, Tokyo 100-8321 (JP)
(74) Representative: Hoffmann Eitle
(86) International application number: PCT/JP2023/010505
(87) International publication number: WO 2023/189696

(57) **Abstract**

Provided is a lubricating oil composition containing: a base oil (A) containing an ester base oil (A1); and a hindered amine compound (B), wherein the content of the component (B) is 0.60 to 10.0 mass% based on the total amount of the lubricating oil composition.

## Description

### Technical Field

The present invention relates to a lubricating oil composition, an internal combustion engine filled with the lubricating oil composition, and a method for using the lubricating oil composition.

### Background Art

In recent years, environmental regulations on a global scale have become increasingly strict, particularly the situation surrounding automobiles, with increasingly stringent fuel economy regulations, exhaust gas regulations, and the like. The background to this is environmental issues such as global warming and resource conservation due to concerns about the depletion of oil resources. Under these recent circumstances, the production ratio of hybrid vehicles, which are powered by an internal combustion engine in combination with an electromotor, has been increasing in order to reduce air pollution caused by exhaust gases from vehicles.

Incidentally, while the same engine oils as the lubricating oils for the internal combustion engine of conventional vehicles powered solely by an internal combustion engine have been used as lubricating oils for the internal combustion engine of hybrid vehicles, the development of lubricating oils for internal combustion engines adapted to the use environment of hybrid vehicles is being pursued.

For example, Patent Literature 1 discloses a lubricating oil composition for internal combustion engines of hybrid vehicles wherein a 100N hydro-refined mineral oil contains a hindered amine compound, an amine antioxidant, a metal-based detergent, and an organic zinc dithiophosphate, and the hindered amine compound and the amine antioxidant are contained at a predetermined ratio.

### Citation List

### Patent Literature

Patent Literature 1: Japanese Patent Laid-Open No. 2016-180069

### Summary of Invention

### Technical Problem

Under these circumstances, there is a need for a lubricating oil composition that can be suitably used for the internal combustion engine of hybrid systems having an internal combustion engine and an electromotor as power sources, with further improved characteristics such as high temperature detergency and long-drain properties.

### Solution to Problem

As a result of extensive studies, the present inventors have found that the above problem can be solved by preparing a lubricating oil composition comprising a predetermined amount of a hindered amine compound with respect to a base oil comprising an ester base oil. Specifically, the present invention discloses the following embodiments.
[1] A lubricating oil composition comprising: a base oil (A) comprising an ester base oil (A1); and a hindered amine compound (B),
   wherein a content of the component (B) is 0.60 to 10.0 mass% based on the total amount of the lubricating oil composition.
[2] An internal combustion engine, which is installed in a hybrid system, and is filled with the lubricating oil composition according to the above [1].
[3] A method for lubricating an internal combustion engine, wherein the lubricating oil composition according to the above [1] is applied to an internal combustion engine installed in a hybrid system.

### Advantageous Effects of Invention

The lubricating oil composition of a preferred embodiment of the present invention has excellent high temperature detergency and long-drain properties, and in a more preferred embodiment, in addition to these characteristics, can retain excellent long-drain properties even when there is water contamination. Therefore, the lubricating oil composition of one embodiment of the present invention can be preferably used for lubrication of the internal combustion engine of a hybrid system.

### Description of Embodiments

Regarding the numerical range described in the present specification, the upper limit and the lower limit can be arbitrarily combined. For example, with the description "preferably 30 to 100, more preferably 40 to 80" as a numerical range, the range of "30 to 80" and the range of "40 to 100" are also included in the numerical range described in the present specification.

In addition, for example, the description of "60 to 100" as the numerical range described in the present specification means a range of "60 or more (60 or more than 60) and 100 or less (100 or less than 100)".

Furthermore, in defining the upper limit values and lower limit values described in the present specification, the numerical range from the lower limit value to the upper limit value can be defined by appropriately selecting from each option and combining them arbitrarily.

In addition, the various requirements described in the present specification as preferred embodiments can be combined in multiple combinations.

In the present specification, the kinematic viscosity and the viscosity index mean values measured and calculated in accordance with JIS K2283:2000.

The content of nitrogen atoms (N) means a value measured in accordance with JIS K2609:1998.

### [Constitution of lubricating oil composition]

The lubricating oil composition of one embodiment of the present invention contains a base oil (A) containing an ester base oil (A1), and a hindered amine compound (B), with the content of the component (B) being 0.60 to 10.0 mass% based on the total amount of the lubricating oil composition.

The present inventors believed that the performance of the hindered amine compound (B) was not sufficiently demonstrated in conventional lubricating oil compositions, and after various studies on means to effectively demonstrate the performance of the hindered amine compound (B), they have found that the high temperature detergency and long-drain properties can be dramatically improved by combining a predetermined amount or more of the hindered amine compound (B) with respect to an ester base oil (A1) as the base oil (A). This effect may be attributed to the high solubility of the hindered amine compound (B) in the ester base oil (A1).

In other words, the lubricating oil composition of one embodiment of the present invention can have dramatically improved high temperature detergency and long-drain properties by using the ester base oil (A1) and the hindered amine compound (B) in combination, and blending 0.60 mass% or more of the hindered amine compound (B).

In addition, the lubricating oil composition of one embodiment of the present invention has the characteristic of being able to retain good long-drain properties even when there is water contamination.

This characteristic is particularly useful for the lubrication of the internal combustion engine of hybrid systems having an internal combustion engine and an electromotor as power sources. For example, compared to the internal combustion engines of conventional vehicles, the internal combustion engines of hybrid vehicles, which are powered by an internal combustion engine and an electromotor, spend more time stopped, even when the vehicle is in use, which can cause condensation to form inside the crankcase. Therefore, the lubricating oil compositions used in hybrid systems such as hybrid vehicles are prone to water contamination, and the water can cause a decrease in long-drain properties.

By contrast, the lubricating oil composition of one embodiment of the present invention more effectively expresses the performance of the hindered amine compound (B), and therefore can retain good long-drain properties even when there is water contamination, which is a factor in degradation.

The lubricating oil composition of one embodiment of the present invention may further contain an antioxidant (C) that does not correspond to the component (B) .

The lubricating oil composition of one embodiment of the present invention may further contain a lubricating oil additive other than the above components (B) to (C) as long as the effects of the present invention are not impaired.

In the lubricating oil composition of one embodiment of the present invention, the total content of the components (A) and (B) is preferably 60 mass% or more, more preferably 65 mass% or more, still more preferably 70 mass% or more, still much more preferably 75 mass% or more, and particularly preferably 80 mass% or more, and may be 100 mass% or less, 99.99 mass% or less, 99.90 mass% or less, 99.50 mass% or less, 99.0 mass% or less, 98.0 mass% or less, 97.0 mass% or less, 95.0 mass% or less, 92.0 mass% or less, or 90.0 mass% or less, based on the total amount (100 mass%) of the lubricating oil composition.

In the lubricating oil composition of one embodiment of the present invention, the total content of the components (A), (B), and (C) is preferably 60 mass% or more, more preferably 65 mass% or more, still more preferably 70 mass% or more, still much more preferably 75 mass% or more, and particularly preferably 80 mass% or more, and may be 100 mass% or less, 99.99 mass% or less, 99.90 mass% or less, 99.50 mass% or less, 99.0 mass% or less, 98.0 mass% or less, 97.0 mass% or less, 95.0 mass% or less, or 92.0 mass% or less, based on the total amount (100 mass%) of the lubricating oil composition.

Details of the components contained in the lubricating oil composition of one embodiment of the present invention will be described hereinafter.

### <Component (A): base oil>

The lubricating oil composition of one embodiment of the present invention contains a base oil (A) containing an ester base oil (A1). By containing the ester base oil (A1), a lubricating oil composition in which the performance of the hindered amine compound (B) is effectively expressed, and with improved high temperature detergency and long-drain properties, can be obtained.

The component (A) used in one embodiment of the present invention may be composed of only the ester base oil (A1), or may be a mixed base oil containing a base oil other than the ester base oil (A1).

In the lubricating oil composition of one embodiment of the present invention, the content of the component (A) is preferably 40 mass% or more, more preferably 50 mass% or more, still more preferably 60 mass% or more, still much more preferably 70 mass% or more, and particularly preferably 80 mass% or more, and may be 99.4 mass% or less, 99.0 mass% or less, 97.0 mass% or less, 95.0 mass% or less, 92.0 mass% or less, or 90.0 mass% or less, based on the total amount (100 mass%) of the lubricating oil composition.

### <Component (A1): ester base oil>

Examples of the component (A1) used in one embodiment of the present invention include one or more selected from polyol esters, diesters, and monoesters.

Of these, from the viewpoint of obtaining a lubricating oil composition in which the performance of the component (B) is more effectively expressed, and with further improved high temperature detergency and long-drain properties, the component (A1) used in one embodiment of the present invention preferably contains one or more selected from a polyol ester (A11) and diester (A12).

From the viewpoint of obtaining a lubricating oil composition in which the performance of the component (B) is more effectively expressed, and with further improved high temperature detergency and long-drain properties, the total content ratio of the components (A11) and (A12) in the component (A1) used in one embodiment of the present invention is preferably 50 to 100 mass%, more preferably 60 to 100 mass%, more preferably 70 to 100 mass%, still more preferably 80 to 100 mass%, still much more preferably 90 to 100 mass%, and particularly preferably 95 to 100 mass%, based on the total amount (100 mass%) of the component (A) contained in the lubricating oil composition.

The polyol ester (A11) used in one embodiment of the present invention may be a full ester or partial ester of a polyol.

The polyol from which the polyol ester (A11) is derived is preferably an aliphatic polyol, and examples thereof include dihydric alcohols such as ethylene glycol, diethylene glycol, triethylene glycol, propylene glycol, trimethylene glycol, tetramethylene glycol, and neopentyl glycol; trihydric alcohols such as glycerol, trimethylolethane, and trimethylolpropane; and polyhydric (tetrahydric or more) alcohols such as diglycerol, triglycerol, pentaerythritol, dipentaerythritol, mannitol, and sorbitol.

The hydrocarbyl group constituting the polyol ester (A11) is preferably an alkyl group or an alkenyl group having 6 to 30 carbon atoms, and more preferably an alkyl group or an alkenyl group having 12 to 24 carbon atoms.

Specific examples of the hydrocarbyl group include a hexyl group, an octyl group, a decyl group, a dodecyl group, a tetradecyl group, a hexadecyl group, a heptadecyl group, an octadecyl group, a hexenyl group, an octenyl group, a decenyl group, a dodecenyl group, a tetradecenyl group, a hexadecenyl group, and an octadecenyl group.

These alkyl and alkenyl groups may be straight-chain alkyl and alkenyl groups or may be branched chain alkyl and alkenyl groups.

Examples of full esters of polyols, which are polyol esters (A11), include neopentyl glycol dilaurate, neopentyl glycol dimyristate, neopentyl glycol dipalmitate, neopentyl glycol distearate, neopentyl glycol diisostearate, trimethylolpropane trilaurate, trimethylolpropane trimyristate, trimethylolpropane tripalmitate, trimethylolpropane tristearate, trimethylolpropane triisostearate, glycerol trilaurate, glycerol tristearate, and glycerol triisostearate.

The partial ester of polyol, which is a polyol ester (A11), has at least one hydroxyl group remaining, and examples thereof include neopentyl glycol monolaurate, neopentyl glycol monomyristate, neopentyl glycol monopalmitate, neopentyl glycol monostearate, neopentyl glycol monoisostearate, trimethylolpropane mono(or di)laurate, trimethylolpropane mono(or di)myristate, trimethylolpropane mono(or di)palmitate, trimethylolpropane mono(or di)stearate, trimethylolpropane mono(or di)isostearate, glycerol mono(or di)laurate, glycerol mono(or di)stearate, and glycerol mono(or di)isostearate.

Examples of the diester (A12) used in one embodiment of the present invention include esters of monohydric alcohols with dibasic acids such as adipic acid, azelaic acid, sebacic acid, and dodecanedioic acid.

The number of carbon atoms of the dibasic acid from which the diester (A12) is derived may be, for example, 4 or more, 5 or more, 6 or more, 8 or more, or 10 or more, and may be 36 or less, 30 or less, 27 or less, 24 or less, or 20 or less.

The number of carbon atoms of the alcohol residue constituting the diester (A12) may be, for example, 1 or more, 4 or more, 6 or more, or 8 or more, and may be 30 or less, 26 or less, 22 or less, or 20 or less.

The kinematic viscosity of the component (A1) used in one embodiment of the present invention at 40°C is preferably 3 to 120 mm²/s, more preferably 5 to 100 mm²/s, still more preferably 7 to 70 mm²/s, still much more preferably 8.5 to 50 mm²/s, and particularly preferably 10 to 30 mm²/s.

The viscosity index of the component (A1) used in one embodiment of the present invention is preferably 70 or more, more preferably 90 or more, still more preferably 100 or more, still much more preferably 110 or more, and particularly preferably 120 or more.

When a mixed oil that is a combination of two or more base oils is used as the component (A1) in one embodiment of the present invention, the kinematic viscosity and the viscosity index of the mixed oil are preferably in the above ranges.

In the lubricating oil composition of one embodiment of the present invention, the content ratio of the component (A1) in the component (A) is, from the viewpoint of obtaining a lubricating oil composition in which the performance of the component (B) is more effectively expressed, and with further improved high temperature detergency and long-drain properties, preferably 10 mass% or more, more preferably 20 mass% or more, more preferably 30 mass% or more, more preferably 40 mass% or more, still more preferably 50 mass% or more, still more preferably 60 mass% or more, still much more preferably 70 mass% or more, and particularly preferably 80 mass% or more, and furthermore, may be 85 mass% or more, 90 mass% or more, or 95 mass% or more, and 100 mass% or less, 97 mass% or less, 95 mass% or less, 92 mass% or less, or 90 mass% or less, based on the total amount (100 mass%) of the component (A) contained in the lubricating oil composition.

In the lubricating oil composition of one embodiment of the present invention, the content of the component (A1) is, from the viewpoint of obtaining a lubricating oil composition in which the performance of the component (B) is more effectively expressed, and with further improved high temperature detergency and long-drain properties, preferably 15 mass% or more, more preferably 25 mass% or more, more preferably 35 mass% or more, still more preferably 45 mass% or more, still more preferably 55 mass% or more, still much more preferably 65 mass% or more, and particularly preferably 75 mass% or more, and may be 99.4 mass% or less, 99.0 mass% or less, 97.0 mass% or less, 95.0 mass% or less, 92.0 mass% or less, or 90.0 mass% or less, based on the total amount (100 mass%) of the lubricating oil composition.

### <Base oil other than component (A1)>

The component (A) used in one embodiment of the present invention may contain a base oil other than the ester base oil (A1).

Examples of the other base oil include one or more selected from mineral oils and synthetic oils other than the component (A1).

Examples of the mineral oils include atmospheric residues obtained by subjecting crude oils, such as paraffinic crude oil, intermediate base crude oil and naphthenic crude oil, to atmospheric distillation; distillates obtained by subjecting these atmospheric residues to vacuum distillation; and refined oils obtained by subjecting the distillates to one or more of refining treatments, such as solvent deasphalting, solvent extraction, hydrocracking, solvent dewaxing, catalytic dewaxing, and hydrorefining.

Examples of the synthetic oils include poly-α-olefins, such as an α-olefin homopolymer and an α-olefin copolymer (for example, an α-olefin copolymer having 8 to 14 carbon atoms such as an ethylene-α-olefin copolymer); isoparaffin; polyalkylene glycol; ether oils, such as polyphenyl ether; alkylbenzene; alkylnaphthalene; and synthetic oil (GTL) obtained by isomerizing wax (GTL WAX (Gas To Liquids WAX)) produced from natural gas through Fischer-Tropsch process or the like.

The base oil other than the component (A1) used in one embodiment of the present invention is preferably one or more selected from mineral oils classified in Group II and Group III of API (American Petroleum Institute) base oil categories, and synthetic oils other than the component (A1).

The kinematic viscosity of the base oil other than the component (A1) used in one embodiment of the present invention at 40°C is preferably 3 to 130 mm²/s, more preferably 5 to 100 mm²/s, still more preferably 7 to 80 mm²/s, still much more preferably 8.5 to 50 mm²/s, and particularly preferably 10 to 30 mm²/s.

The viscosity index of the base oil other than the component (A1) used in one embodiment of the present invention is preferably 70 or more, more preferably 90 or more, still more preferably 100 or more, still much more preferably 110 or more, and particularly preferably 120 or more.

When a mixed oil that is a combination of two or more base oils is used as the other base oil in one embodiment of the present invention, the kinematic viscosity and the viscosity index of the mixed oil are preferably in the above ranges.

The base oil other than component (A1) used in one embodiment of the present invention can also be selected in accordance with the properties to be imparted to the lubricating oil composition. For example, a mineral oil (A2) is preferably contained from the viewpoint of obtaining a lubricating oil composition that can effectively suppress the swelling of resin materials.

In the lubricating oil composition of one embodiment of the present invention, when the component (A) contains an ester base oil (A1) and a mineral oil (A2), the content ratio by mass of the component (A1) to the component (A2), [(A1)/(A2)], may be, from the viewpoint of obtaining a lubricating oil composition in which the performance of the component (B) is more effectively expressed, and with further improved high temperature detergency and long-drain properties, 10/90 or more, 15/85 or more, 20/80 or more, 25/75 or more, 30/70 or more, 35/65 or more, 40/60 or more, 45/55 or more, 50/50 or more, 55/45 or more, 60/40 or more, 65/35 or more, 70/30 or more, 75/25 or more, or 80/20 or more, and from the viewpoint of obtaining a lubricating oil composition that can effectively suppress the swelling of resin materials, it may be 99/1 or less, 95/5 or less, 90/10 or less, 85/15 or less, 80/20 or less, 75/25 or less, 70/30 or less, 65/35 or less, 60/40 or less, 55/45 or less, 50/50 or less, 45/55 or less, 40/60 or less, 35/65 or less, or 30/70 or less.

In the lubricating oil composition of one embodiment of the present invention, the content ratio of the component (A2) in the component (A) is, from the viewpoint of obtaining a lubricating oil composition in which the performance of the component (B) is more effectively expressed, and with further improved high temperature detergency and long-drain properties, preferably 90 mass% or less, more preferably 80 mass% or less, more preferably 70 mass% or less, more preferably 60 mass% or less, still more preferably 50 mass% or less, still more preferably 40 mass% or less, still much more preferably 30 mass% or less, and particularly preferably 20 mass% or less, and furthermore, may be 15 mass% or less, 10 mass% or less, 5 mass% or less, less than 2 mass%, or less than 1 mass%, and 0 mass% or more, more than 0 mass%, 1 mass% or more, 3 mass% or more, 5 mass% or more, 8 mass% or more, or 10 mass% or more, based on the total amount (100 mass%) of the component (A) contained in the lubricating oil composition.

In the lubricating oil composition of one embodiment of the present invention, the content of the component (A2) may be 0 mass% or more, more than 0 mass%, 1 mass% or more, 5 mass% or more, 10 mass% or more, 15 mass% or more, 20 mass% or more, 25 mass% or more, or 30 mass% or more, and may be 65 mass% or less, 60 mass% or less, 55 mass% or less, 50 mass% or less, 45 mass% or less, 40 mass% or less, 35 mass% or less, 30 mass% or less, 25 mass% or less, 20 mass% or less, 15 mass% or less, 10 mass% or less, 5 mass% or less, less than 2 mass%, or less than 1 mass%, based on the total amount (100 mass%) of the lubricating oil composition.

### <Component (B): hindered amine compound>

The lubricating oil composition of one embodiment of the present invention contains 0.60 to 10.0 mass% of a hindered amine compound as the component (B) based on the total amount of the lubricating oil composition.

Because it contains 0.60 mass% or more of the hindered amine compound (B), the lubricating oil composition of one embodiment of the present invention can have dramatically improved high temperature detergency and long-drain properties, and in particular, can retain good long-drain properties even when there is water contamination, which is a factor in degradation. On the other hand, when the content of the component (B) is less than 0.60 mass%, it becomes difficult to sufficiently improve the long-drain properties particularly when there is water contamination. In addition, when the content of the component (B) is more than 10.0 mass%, the high temperature detergency may decrease.

The component (B) used in one embodiment of the present invention may be used singly, or may be used in combination of two or more.

In the lubricating oil composition of one embodiment of the present invention, the content of the component (B) is, from the viewpoint of obtaining a lubricating oil composition with better long-drain properties even when there is water contamination, preferably 0.70 mass% or more, more preferably 1.00 mass% or more, more preferably 1.20 mass% or more, more preferably 1.50 mass% or more, more preferably 1.70 mass% or more, still more preferably 2.00 mass% or more, still more preferably 2.20 mass% or more, still more preferably 2.50 mass% or more, still more preferably 3.00 mass% or more, still much more preferably 4.00 mass% or more, still much more preferably 5.00 mass% or more, and particularly preferably 5.50 mass% or more, and from the viewpoint of obtaining a lubricating oil composition with good high temperature detergency, it is preferably 10.0 mass% or less, more preferably 9.50 mass% or less, more preferably 9.00 mass% or less, still more preferably 8.50 mass% or less, still more preferably 8.00 mass% or less, still much more preferably 7.5 mass% or less, and particularly preferably 7.00 mass% or less, based on the total amount (100 mass%) of the lubricating oil composition.

The content of the component (B) in terms of nitrogen atoms in the lubricating oil composition of one embodiment of the present invention is, from the viewpoint of obtaining a lubricating oil composition with better long-drain properties even when there is water contamination, preferably more than 0.05 mass%, more preferably 0.07 mass% or more, more preferably 0.10 mass% or more, still more preferably 0.12 mass% or more, still more preferably 0.15 mass% or more, still much more preferably 0.17 mass% or more, and particularly preferably 0.20 mass% or more, and from the viewpoint of obtaining a lubricating oil composition with good high temperature detergency, it is preferably 0.60 mass% or less, more preferably 0.50 mass% or less, more preferably 0.45 mass% or less, more preferably 0.42 mass% or less, still more preferably 0.40 mass% or less, still more preferably 0.37 mass% or less, still more preferably 0.35 mass% or less, still much more preferably 0.32 mass% or less, and particularly preferably 0.30 mass% or less, based on the total amount (100 mass%) of the lubricating oil composition.

In the lubricating oil composition of one embodiment of the present invention, the content of the component (B) based on the total 100 parts by mass of the component (A) is, from the viewpoint of obtaining a lubricating oil composition with better long-drain properties even when there is water contamination, preferably 1.0 part by mass or more, more preferably 1.5 parts by mass or more, more preferably 2.0 parts by mass or more, more preferably 2.5 parts by mass or more, more preferably 3.0 parts by mass or more, still more preferably 3.5 parts by mass or more, still more preferably 4.0 parts by mass or more, still more preferably 4.5 parts by mass or more, still more preferably 5.0 parts by mass or more, still much more preferably 5.5 parts by mass or more, and particularly preferably 6.0 parts by mass or more, and it is preferably 50.0 parts by mass or less, more preferably 40.0 parts by mass or less, more preferably 30.0 parts by mass or less, more preferably 25.0 parts by mass or less, more preferably 20.0 parts by mass or less, still more preferably 18.0 parts by mass or less, still more preferably 16.0 parts by mass or less, still more preferably 14.0 parts by mass or less, still more preferably 12.0 parts by mass or less, still much more preferably 10.0 parts by mass or less, and particularly preferably 9.0 parts by mass or less.

In the lubricating oil composition of one embodiment of the present invention, the content of the component (B) based on the total 100 parts by mass of the component (A1) is, from the viewpoint of obtaining a lubricating oil composition with better long-drain properties even when there is water contamination, preferably 2.5 parts by mass or more, more preferably 3.0 parts by mass or more, more preferably 3.5 parts by mass or more, still more preferably 4.0 parts by mass or more, still more preferably 4.5 parts by mass or more, still much more preferably 5.0 parts by mass or more, still much more preferably 5.5 parts by mass or more, and particularly preferably 6.0 parts by mass or more, and it is preferably 50.0 parts by mass or less, more preferably 40.0 parts by mass or less, more preferably 30.0 parts by mass or less, more preferably 25.0 parts by mass or less, more preferably 20.0 parts by mass or less, still more preferably 18.0 parts by mass or less, still more preferably 16.0 parts by mass or less, still more preferably 14.0 parts by mass or less, still more preferably 12.0 parts by mass or less, still much more preferably 10.0 parts by mass or less, and particularly preferably 9.0 parts by mass or less.

In one embodiment of the present invention, the hindered amine compound used as the component (B) may be a compound containing the structure represented by the following formula (b-0).

In the above formula, *1 and *2 represent a position of bonding with another atom.

The component (B) used in one embodiment of the present invention preferably contains one or more selected from a compound (B1) represented by the following general formula (b-1) and a compound (B2) represented by the following general formula (b-2).

In the above general formulae (b-1) and (b-2), R^{b1} is each independently a hydrogen atom, an alkyl group having 1 to 10 carbon atoms, or an alkoxy group having 1 to 10 carbon atoms.

In the above general formula (b-1), R^{b2} is a hydrogen atom, an alkyl group having 1 to 20 carbon atoms, a cycloalkyl group having 3 to 18 ring-forming carbon atoms, an aryl group having 6 to 18 ring-forming carbon atoms, a hydroxyl group, an amino group, or a group represented by -O-CO-R^{b3} (R^{b3} is a hydrogen atom or a hydrocarbon group having 1 to 20 carbon atoms).

In the above general formula (b-2), Z is an alkylene group having 1 to 20 carbon atoms, a cycloalkylene group having 3 to 18 ring-forming carbon atoms, an arylene group having 6 to 18 ring-forming carbon atoms, an oxygen atom, a sulfur atom, or a group represented by -O-CO-(CH₂)ₙ-CO-O- (n is an integer of 1 to 20) .

Examples of the alkyl groups that can be selected as R^{b1} include a methyl group, an ethyl group, a propyl group (n-propyl group and isopropyl group), a butyl group (n-butyl group, s-butyl group, t-butyl group, isobutyl group), a pentyl group, a hexyl group, a 2-ethylhexyl group, a heptyl group, an octyl group, a nonyl group, and a decyl group. These alkyl groups may be straight-chain alkyl groups or may be branched chain alkyl groups.

The number of carbon atoms of the alkyl groups that can be selected as R^{b1} is preferably 1 to 10, more preferably 1 to 6, and still more preferably 1 to 3.

Examples of the alkoxy groups that can be selected as R^{b1} include a methoxy group, an ethoxy group, a propoxy group (n-propoxy group and isopropoxy group), a butoxy group (n-butoxy group, s-butoxy group, t-butoxy group, and isobutoxy group), a pentyloxy group, a hexyloxy group, a 2-ethylhexyloxy group, a heptyloxy group, an octyloxy group, a nonyloxy group, a decyloxy group, and a group represented by -(CH₂)ₙ- (n is an integer of 1 to 20). These alkoxy groups may be straight-chain alkoxy groups or may be branched chain alkoxy groups.

The number of carbon atoms of the alkoxy groups that can be selected as R^{b1} is preferably 1 to 10, more preferably 1 to 6, and still more preferably 1 to 3.

Examples of the alkyl groups that can be selected as R^{b2} include the aforementioned alkyl groups having 1 to 10 carbon atoms that can be selected as R^{b1}, as well as an undecyl group, a dodecyl group, a tridecyl group, a tetradecyl group, a hexadecyl group, and an octadecyl group. These alkyl groups may be straight-chain alkyl groups or may be branched chain alkyl groups.

The number of carbon atoms of the alkyl groups that can be selected as R^{b2} is preferably 1 to 20, more preferably 3 to 18, still more preferably 6 to 16, and still much more preferably 8 to 14.

Examples of the cycloalkyl groups that can be selected as R^{b2} include a cyclopropyl group, a cyclobutyl group, a cyclopentyl group, a cyclohexyl group, a cycloheptyl group, a cyclooctyl group, and an adamantyl group.

The number of ring-forming carbon atoms of the cycloalkyl groups that can be selected as R^{b2} is preferably 3 to 18, more preferably 5 to 15, and still more preferably 6 to 12.

Examples of the aryl groups that can be selected as R^{b2} include a phenyl group, a naphthyl group, an anthryl group, a phenanthryl group, a biphenyl group, a terphenyl group, and a phenylnaphthyl group.

The number of ring-forming carbon atoms of the aryl groups that can be selected as R^{b2} is preferably 6 to 18, more preferably 6 to 15, and still more preferably 6 to 12.

Examples of the alkylene groups that can be selected as Z include a methylene group, a 1,1-ethylene group, a 1,2-ethylene group, various propylene groups such as 1,3-propylene, 1,2-propylene, and 2,2-propylene, various butylene groups, various pentylene groups, various hexylene groups, various heptylene groups, various octylene groups, various nonylene groups, various decylene groups, various undecylene groups, various dodecylene groups, various tridecylene groups, various tetradecylene groups, various pentadecylene groups, various hexadecylene groups, various heptadecylene groups, and various octadecylene groups.

Examples of the cycloalkylene groups that can be selected as Z include a cyclopropylene group, a cyclobutylene group, a cyclopentylene group, a cyclohexylene group, a cycloheptylene group, a cyclooctylene group, and an adamantylene group.

Examples of the arylene groups that can be selected as Z include a phenylene group, a naphthylene group, an anthrylene group, a phenanthrylene group, a biphenylene group, and a terphenylene group.

The component (B) used in one embodiment of the present invention more preferably contains one or more selected from a compound (B11) represented by the following general formula (b-11) and a compound (B21) represented by the following general formula (b-21).

In the above general formulae (b-11) and (b-21), R^{b1} is each independently a hydrogen atom or an alkyl group having 1 to 10 carbon atoms. Specific examples of the alkyl groups that can be selected as R^{b1} and the preferred range of the number of carbon atoms is as previously described.

In the above general formula (b-11), R^{b3} is a hydrogen atom or a hydrocarbon group having 1 to 20 carbon atoms.

In the above general formula (b-21), n is an integer of 1 to 20.

Examples of the hydrocarbon groups that can be selected as R^{b3} include an alkyl group having 1 to 20 carbon atoms, an alkenyl group having 2 to 20 carbon atoms, a cycloalkyl group having 3 to 18 ring-forming carbon atoms optionally substituted with an alkyl group having 1 to 10 carbon atoms, an aryl group having 6 to 18 ring-forming carbon atoms optionally substituted with an alkyl group having 1 to 10 carbon atoms, and an arylalkyl group having 7 to 19 carbon atoms.

The alkyl groups may be straight-chain alkyl groups or may be branched chain alkyl groups. The alkenyl groups may be straight-chain alkenyl groups or may be branched chain alkenyl groups.

Examples of the alkyl groups, cycloalkyl groups and aryl groups that can be selected as R^{b3} include the same groups as the alkyl groups, cycloalkyl groups and aryl groups that can be selected as R^{b2}.

Examples of the alkenyl groups that can be selected as R^{b3} include an ethenyl group (vinyl group), a propenyl group, a butenyl group, a pentenyl group, a hexenyl group, a heptenyl group, an octenyl group, a nonenyl group, a decenyl group, a dodecenyl group, a tridecenyl group, a tetradecenyl group, a pentadecenyl group, a hexadecenyl group, and an octadecenyl group (oleyl group) .

Examples of the arylalkyl groups that can be selected as R^{b3} include a phenylmethyl group, a phenylethyl group, a naphthylmethyl group, and a naphthylethyl group.

Of these, R^{b3} is preferably an alkyl group having 1 to 20 carbon atoms or an alkenyl group having 2 to 20 carbon atoms, and more preferably an alkyl group having 1 to 20 carbon atoms.

The number of carbon atoms of the alkyl groups that can be selected as R^{b3} is preferably 3 to 20, more preferably 4 to 18, still more preferably 6 to 16, and still much more preferably 8 to 14.

The number of carbon atoms of the alkenyl groups that can be selected as R^{b3} is preferably 2 to 20, more preferably 3 to 18, and still more preferably 6 to 16.

The component (B) used in one embodiment of the present invention preferably contains at least a compound (B1) represented by the general formula (b-1), and more preferably contains at least a compound (B11) represented by the general formula (b-11).

In the lubricating oil composition of one embodiment of the present invention, the content ratio of the component (B1) or (B11) in the component (B) is preferably 40 to 100 mass% or more, more preferably 50 to 100 mass%, more preferably 60 to 100 mass%, still more preferably 70 to 100 mass%, still more preferably 80 to 100 mass%, still much more preferably 90 to 100 mass%, and particularly preferably 95 to 100 mass%, based on the total amount (100 mass%) of the component (B) contained in the lubricating oil composition, from the viewpoint of obtaining a lubricating oil composition having further improved high temperature detergency and long-drain properties.

### <Component (C): antioxidant that does not correspond to the component (B)>

From the viewpoint of obtaining a lubricating oil composition having further improved high temperature detergency and long-drain properties, the lubricating oil composition of one embodiment of the present invention may contain an antioxidant that does not correspond to the component (B) as the component (C).

Examples of the component (C) used in one embodiment of the present invention include an amine antioxidant other than a hindered amine compound, a phenolic antioxidant, a sulfur antioxidant, and a phosphorus antioxidant.

The component (C) may be used singly, or may be used in combination of two or more.

The component (C) used in one embodiment of the present invention preferably contains one or more selected from an amine antioxidant (C1) other than a hindered amine compound and a phenolic antioxidant (C2), and more preferably contains both component (C1) and component (C2).

The total content ratio of the components (C1) and (C2) in the component (C) used in one embodiment of the present invention is preferably 60 to 100 mass%, more preferably 70 to 100 mass%, more preferably 80 to 100 mass%, still more preferably 85 to 100 mass%, still much more preferably 90 to 100 mass%, and particularly preferably 95 to 100 mass%, based on the total amount (100 mass%) of the component (C) contained in the lubricating oil composition.

When the component (C) used in one embodiment of the present invention contains both components (C1) and (C2), the content ratio by mass of the component (C1) to the component (C2), [(C1)/(C2)], is preferably 0.10 to 5.0, more preferably 0.15 to 3.0, more preferably 0.20 to 1.0, still more preferably 0.25 to 0.90, still much more preferably 0.30 to 0.80, and particularly preferably 0.35 to 0.70.

Examples of the component (C1) used in one embodiment of the present invention include a diphenylamine antioxidant, such as diphenylamine, and alkylated diphenylamine having an alkyl group with 3 to 20 (preferably 6 to 16, more preferably 8 to 12) carbon atoms; and a naphthylamine antioxidant such as α-naphthylamine, phenyl-α-naphthylamine, and substituted phenyl-α-naphthylamine having an alkyl group with 3 to 20 (preferably 6 to 16, more preferably 8 to 12) carbon atoms.

Examples of the component (C2) used in one embodiment of the present invention include a monophenolic antioxidant such as 2,6-di-t-butylphenol, 2,6-di-t-butyl-4-methylphenol, 2,6-di-t-butyl-4-ethylphenol, isooctyl-3-(3,5-di-t-butyl-4-hydroxyphenyl)propionate, octadecyl-3-(3,5-di-t-butyl-4-hydroxyphenyl)propionate, and benzenepropanoic acid-3,5-bis(1,1-dimethylethyl)-4-hydroxyalkyl ester; and a diphenolic antioxidant such as 4,4'-methylenebis(2,6-dit-butylphenol), 2,2'-methylenebis(4-ethyl-6-t-butylphenol) and thiodiethylenebis[3-(3,5-di-t-butyl-4-hydroxyphenyl)propionate].

In the lubricating oil composition of one embodiment of the present invention, the content of the component (C) is preferably 0.01 mass% or more, more preferably 0.05 mass% or more, more preferably 0.10 mass% or more, still more preferably 0.30 mass% or more, still more preferably 0.50 mass% or more, still much more preferably 0.60 mass% or more, and particularly preferably 0.70 mass% or more, and furthermore, may be 0.75 mass% or more, 0.80 mass% or more, 0.85 mass% or more, or 0.90 mass% or more, and 10.0 mass% or less, 8.0 mass% or less, 6.0 mass% or less, 5.0 mass% or less, 4.0 mass% or less, 3.0 mass% or less, or 2.0 mass% or less, based on the total amount (100 mass%) of the lubricating oil composition.

In the lubricating oil composition of one embodiment of the present invention, the content of the component (C) based on the total 100 parts by mass of the component (B) is preferably 1.0 part by mass or more, more preferably 3.0 parts by mass or more, more preferably 5.0 parts by mass or more, still more preferably 7.0 parts by mass or more, still more preferably 10 parts by mass or more, still much more preferably 12 parts by mass or more, and particularly preferably 14 parts by mass or more, and it is preferably 100 parts by mass or less, more preferably 80 parts by mass or less, more preferably 60 parts by mass or less, still more preferably 50 parts by mass or less, still much more preferably 40 parts by mass or less, still much more preferably 35 parts by mass or less, and particularly preferably 30 parts by mass or less.

In the lubricating oil composition of one embodiment of the present invention, the content of the component (C1) is preferably 0.01 mass% or more, more preferably 0.05 mass% or more, still more preferably 0.10 mass% or more, still much more preferably 0.15 mass% or more, and particularly preferably 0.20 mass% or more, and may be 5.0 mass% or less, 4.0 mass% or less, 3.0 mass% or less, 2.0 mass% or less, 1.0 mass% or less, 0.80 mass% or less, 0.60 mass% or less, or 0.40 mass% or less, based on the total amount (100 mass%) of the lubricating oil composition.

In the lubricating oil composition of one embodiment of the present invention, the content of the component (C1) in terms of nitrogen atoms is preferably 0.001 mass% or more, more preferably 0.003 mass% or more, still more preferably 0.005 mass% or more, still much more preferably 0.007 mass% or more, and particularly preferably 0.009 mass% or more, and may be 1.0 mass% or less, 0.50 mass% or less, 0.20 mass% or less, 0.10 mass% or less, 0.08 mass% or less, 0.05 mass% or less, or 0.03 mass% or less, based on the total amount (100 mass%) of the lubricating oil composition.

In the lubricating oil composition of one embodiment of the present invention, the content of the component (C1) based on the total 100 parts by mass of the component (B) is preferably 0.1 parts by mass or more, more preferably 1.0 part by mass or more, more preferably 2.0 parts by mass or more, still more preferably 3.0 parts by mass or more, still much more preferably 4.0 parts by mass or more, and particularly preferably 5.0 parts by mass or more, and it is preferably 50 parts by mass or less, more preferably 40 parts by mass or less, more preferably 30 parts by mass or less, still more preferably 20 parts by mass or less, still much more preferably 15 parts by mass or less, still much more preferably 9.0 parts by mass or less, and particularly preferably 7.5 parts by mass or less.

In the lubricating oil composition of one embodiment of the present invention, the content of the component (C2) is preferably 0.01 mass% or more, more preferably 0.05 mass% or more, more preferably 0.10 mass% or more, still more preferably 0.20 mass% or more, still much more preferably 0.30 mass% or more, and particularly preferably 0.40 mass% or more, and may be 5.0 mass% or less, 4.0 mass% or less, 3.0 mass% or less, 2.0 mass% or less, or 1.0 mass% or less, based on the total amount (100 mass%) of the lubricating oil composition.

In the lubricating oil composition of one embodiment of the present invention, the content of the component (C2) based on the total 100 parts by mass of the component (B) is preferably 1.0 part by mass or more, more preferably 3.0 parts by mass or more, more preferably 5.0 parts by mass or more, still more preferably 7.0 parts by mass or more, still much more preferably 9.0 parts by mass or more, and particularly preferably 10.0 parts by mass or more, and it is preferably 60 parts by mass or less, more preferably 50 parts by mass or less, more preferably 40 parts by mass or less, still more preferably 30 parts by mass or less, still much more preferably 25 parts by mass or less, still much more preferably 20 parts by mass or less, and particularly preferably 16 parts by mass or less.

### <Metal-based detergent>

The lubricating oil composition of one embodiment of the present invention may or may not further contain a metal-based detergent.

If a metal-based detergent is contained, the metal-based detergent may be used singly, or may be used in combination of two or more.

Examples of the metal-based detergent used in one embodiment of the present invention include metal salt compounds of organic acids containing a metal atom selected from alkali metals and alkaline earth metals, with specific examples including metal salicylates, metal phenates, and metal sulfonates containing a metal atom selected from alkali metals and alkaline earth metals.

The metal atom contained in the metal-based detergent is preferably sodium, calcium, magnesium, or barium, and more preferably calcium, from the viewpoint of obtaining a lubricating oil composition having further improved high temperature detergency.

In one embodiment of the present invention, the metal-based detergent may be either a neutral salt, a basic salt, an overbased salt, or a mixture thereof.

The total base number of the metal-based detergent is preferably 0 to 600 mg KOH/g.

In one embodiment of the present invention, if the metal-based detergent is a basic salt or an overbased salt, the total base number of the metal-based detergent is preferably 10 to 600 mg KOH/g, more preferably 20 to 500 mg KOH/g.

In the present specification, the "base number" means a base number measured by perchloric acid method in accordance with JIS K2501 "Petroleum products and lubricants - Determination of neutralization number", 7.

In the lubricating oil composition of one embodiment of the present invention, the content of the metal-based detergent in terms of metal atoms may be 50 ppm by mass or more, 100 ppm by mass or more, or 150 ppm by mass or more, and may be 3000 ppm by mass or less, 1000 ppm by mass or less, 700 ppm by mass or less, 500 ppm by mass or less, or 400 ppm by mass or less, based on the total amount (100 mass%) of the lubricating oil composition.

Generally, by containing a metal-based detergent, the high temperature detergency of the lubricating oil composition can be improved. However, since the lubricating oil composition of one embodiment of the present invention contains 0.60 mass% or more of the component (B), which is sufficiently dissolved by using the component (A), excellent high temperature detergency can be exhibited even if the content of the metal-based detergent is small or nil. In addition, as the metal-based detergent can be a factor in the decrease in long-drain properties (particularly the decrease in long-drain properties when there is water contamination), the content of the metal-based detergent is preferably as small as possible from the viewpoint of having good long-drain properties.

From the viewpoint of obtaining a lubricating oil composition with better long-drain properties even when there is water contamination, the content of the metal-based detergent in terms of metal atoms in the lubricating oil composition of one embodiment of the present invention is preferably less than 50 ppm by mass, more preferably less than 40 ppm by mass, more preferably less than 30 ppm by mass, still more preferably less than 20 ppm by mass, still more preferably less than 10 ppm by mass, still much more preferably less than 5 ppm by mass, and particularly preferably less than 2 ppm by mass, based on the total amount (100 mass%) of the lubricating oil composition.

Even if the content of the metal-based detergent is limited as described above, since the lubricating oil composition of one embodiment of the present invention contains 0.60 mass% or more of the component (B), which is sufficiently dissolved by using the component (A), excellent high temperature detergency can be exhibited.

In the present specification, the content of metal atoms such as alkali metal atoms and alkaline earth metal atoms mean values measured in accordance with JPI-5S-38-92.

### <Lubricating oil additive>

The lubricating oil composition of one embodiment of the present invention may further contain other lubricating oil additive other than the components (B) to (C) when needed as long as the effects of the present invention are not impaired.

Examples of such lubricating oil additives include a pour point depressant, a viscosity index improver, a friction modifier, an anti-wear agent, an extreme pressure agent, a metal deactivator, an oil agent, an ashless dispersant, an anti-rust agent, and an anti-foaming agent.

These lubricating oil additives may be each used singly, or may be each used in combination of two or more.

The contents of these lubricating oil additives can be each appropriately adjusted as long as the effects of the present invention are not impaired, and the contents of the additives are each independently usually 0.001 to 15 mass%, preferably 0.005 to 10 mass%, and more preferably 0.01 to 5 mass%, based on the total amount (100 mass%) of the lubricating oil composition.

### [Pour point depressant]

The lubricating oil composition of one embodiment of the present invention may further contain a pour point depressant. The pour point depressant may be used singly, or may be used in combination of two or more.

Examples of the pour point depressants used in one embodiment of the present invention include an ethylenevinyl acetate copolymer, a condensate of chlorinated paraffin and naphthalene, a condensate of chlorinated paraffin and phenol, polymethacrylate, and polyalkylstyrene.

The mass-average molecular weight (Mw) of the pour point depressant used in one embodiment of the present invention may be 5,000 or more, 7,000 or more, 10,000 or more, 15,000 or more, 20,000 or more, 25,000 or more, 30,000 or more, 35,000 or more, 40,000 or more, 45,000 or more, 50,000 or more, 55,000 or more, or 60,000 or more, and may be 150,000 or less, 120,000 or less, 100,000 or less, 90,000 or less, or 80,000 or less.

### [Viscosity index improver]

The lubricating oil composition of one embodiment of the present invention may further contain a viscosity index improver. The viscosity index improver may be used singly, or may be used in combination of two or more.

Examples of the viscosity index improvers used in one embodiment of the present invention include polymers such as non-dispersed polymethacrylate, dispersed polymethacrylate, an olefin copolymer (e.g., ethylene-propylene copolymer), a dispersed olefin copolymer, and a styrene copolymer (e.g., styrene-diene copolymer and styrene-isoprene copolymer).

The weight-average molecular weight (Mw) of the viscosity index improver used in one embodiment of the present invention may be 5,000 or more, 7,000 or more, 10,000 or more, 15,000 or more, or 20,000 or more, and may be 1,000,000 or less, 700,000 or less, 500,000 or less, 300,000 or less, 200,000 or less, 100,000 or less, or 50,000 or less.

### [Friction modifier and anti-wear agent]

The lubricating oil composition of one embodiment of the present invention may further contain a friction modifier or an anti-wear agent. The friction modifier or anti-wear agent may be used singly, or may be used in combination of two or more.

Examples of the friction modifiers and anti-wear agents used in one embodiment of the present invention include sulfur compounds such as a sulfurized olefin, a dialkyl polysulfide, a diarylalkyl polysulfide, and a diaryl polysulfide; phosphorous compounds such as a phosphoric acid ester, a thiophosphoric acid ester, a phosphorous acid ester, an alkylhydrogen phosphite, an amine salt of phosphoric acid ester, and an amine salt of phosphorous acid ester; organic molybdenum compounds such as molybdenum dithiocarbamate (MoDTC), molybdenum dithiophosphate (MoDTP), and an amine salt of molybdic acid; organic zinc compounds such as zinc dithiophosphate (ZnDTP) and zinc dithiocarbamate (ZnDTC); and ashless friction modifiers such as an amine compound, a fatty acid ester, a fatty acid amide, a fatty acid, an aliphatic alcohol, an aliphatic ether, an urea compound, and a hydrazide compound.

### [Extreme pressure agent]

The lubricating oil composition of one embodiment of the present invention may further contain an extreme pressure agent. The extreme pressure agent may be used singly, or may be used in combination of two or more.

Examples of the extreme pressure agents used in one embodiment of the present invention include sulfur compounds such as a sulfurized olefin, a dialkyl polysulfide, a diarylalkyl polysulfide, and a diaryl polysulfide; and phosphorous compounds such as a phosphoric acid ester, a thiophosphoric acid ester, a phosphorous acid ester, an alkylhydrogen phosphite, an amine salt of phosphoric acid ester, and an amine salt of phosphorous acid ester.

### [Metal deactivator]

The lubricating oil composition of one embodiment of the present invention may further contain a metal deactivator. The metal deactivator may be used singly, or may be used in combination of two or more.

Examples of the metal deactivators used in one embodiment of the present invention include benzotriazole, a triazole derivative, a benzotriazole derivative, and a thiadiazole derivative.

### [Oil agent]

The lubricating oil composition of one embodiment of the present invention may further contain an oil agent. The oil agent may be used singly, or may be used in combination of two or more.

Examples of the oil agents used in one embodiment of the present invention include aliphatic saturated and unsaturated monocarboxylic acids such as stearic acid and oleic acid; polymerized fatty acids such as a dimer acid and a hydrogenated dimer acid; hydroxy fatty acids such as ricinoleic acid and 12-hydroxystearic acid; aliphatic saturated and unsaturated monoalcohols such as a lauryl alcohol and an oleyl alcohol; aliphatic saturated and unsaturated monoamines such as a stearylamine and an oleylamine; and aliphatic saturated and unsaturated monocarboxylic acid amides such as a lauramide and an oleamide.

### [Ashless dispersant]

The lubricating oil composition of one embodiment of the present invention may further contain an ashless dispersant from the viewpoint of having good dispersing ability. The ashless dispersant may be used singly, or may be used in combination of two or more.

The ashless dispersant used in one embodiment of the present invention is preferably an alkenyl succinimide, and examples thereof include an alkenyl bis-succinimide represented by the following general formula (f-1) and an alkenyl monosuccinimide represented by the following general formula (f-2).

In the above general formulae (f-1) and (f-2), R^{f1}, R^{f2} and R^{f3} are each independently an alkenyl group having a mass-average molecular weight (Mw) of 500 to 3000 (preferably 900 to 2500).

Examples of the alkenyl groups that can be selected as R^{f1}, R^{f2} and R^{f3} include a polybutenyl group, a polyisobutenyl group, and an ethylene-propylene copolymer, and among these, a polybutenyl group or a polyisobutenyl group is preferable.

A^{f1}, A^{f2} and A^{f3} are each independently an alkylene group having 2 to 5 carbon atoms.
x1 is an integer of 0 to 10, preferably an integer of 1 to 4, and more preferably 2 or 3.
x2 is an integer of 1 to 10, preferably an integer of 2 to 5, and more preferably 3 or 4.

The compound represented by the aforementioned general formula (f-1) or (f-2) may be a modified alkenyl succinimide reacted with one or more selected from a boron compound, an alcohol, an aldehyde, a ketone, an alkylphenol, a cyclic carbonate, an epoxy compound, an organic acid, and the like.

### [Anti-rust agent]

The lubricating oil composition of one embodiment of the present invention may further contain an anti-rust agent. The anti-rust agent may be used singly, or may be used in combination of two or more.

Examples of the anti-rust agents used in one embodiment of the present invention include a fatty acid, an alkenyl succinic acid half ester, a fatty acid soap, an alkyl sulfonic acid salt, a polyhydric alcohol fatty acid ester, a fatty acid amine, oxidized paraffin, and an alkyl polyoxyethylene ether.

### [Anti-foaming agent]

The lubricating oil composition of one embodiment of the present invention may further contain an anti-foaming agent. The anti-foaming agent may be used singly, or may be used in combination of two or more.

Examples of the anti-foaming agents used in one embodiment of the present invention include an alkyl silicone anti-foaming agent, a fluorosilicone anti-foaming agent, and a fluoroalkyl ether anti-foaming agent.

### <Method for producing lubricating oil composition>

The method for producing a lubricating oil composition of one embodiment of the present invention is not particularly limited, but from the viewpoint of productivity, the method is preferably a method having a step of adding the aforementioned component (B), and if needed, the components (C) to (D) and the other lubricating oil additives, to the base oil (A).

### [Properties of lubricating oil composition]

The kinematic viscosity of the lubricating oil composition of one embodiment of the present invention at 40°C is preferably 10 to 120 mm²/s, more preferably 15 to 100 mm²/s, still more preferably 20 to 80 mm²/s, still much more preferably 25 to 70 mm²/s, and particularly preferably 27 to 60 mm²/s.

The kinematic viscosity of the lubricating oil composition of one embodiment of the present invention at 100°C is preferably 2.5 to 20.0 mm²/s, more preferably 4.0 to 18.0 mm²/s, still more preferably 5.0 to 16.0 mm²/s, still much more preferably 6.0 to 14.0 mm²/s, and particularly preferably 7.0 to 12.0 mm²/s.

The viscosity index of the lubricating oil composition of one embodiment of the present invention is preferably 80 or more, more preferably 100 or more, more preferably 120 or more, still more preferably 150 or more, still much more preferably 170 or more, and particularly preferably 200 or more.

The oxidation induction time (OIT) for the lubricating oil composition of one embodiment of the present invention, as measured by performing a test for evaluating the long-drain properties as described in Examples described later, is preferably 50 minutes or more, more preferably 60 minutes or more, more preferably 70 minutes or more, still more preferably 90 minutes or more, still more preferably 100 minutes or more, still much more preferably 120 minutes or more, and particularly preferably 150 minutes or more.

The merit rating for the lubricating oil composition of one embodiment of the present invention, obtained by performing a hot tube test as described in Examples described later and evaluating the degree of color change, is preferably 7.0 or more, more preferably 7.5 or more, more preferably 8.0 or more, still more preferably 8.5 or more, still much more preferably 9.0 or more, and particularly preferably 9.5 or more.

### [Use application of lubricating oil composition]

The lubricating oil composition of one embodiment of the present invention has excellent high temperature detergency and long-drain properties, and in addition to these characteristics, can retain excellent long-drain properties even when there is water contamination.

Therefore, the lubricating oil composition of one embodiment of the present invention can be applied to various apparatuses that can exhibit the above characteristics, but it can be suitably used for lubrication between parts in an internal combustion engine, and particularly for lubrication between parts in an internal combustion engine of a hybrid system having an internal combustion engine and an electromotor as power sources.

When the aforementioned characteristics of the lubricating oil composition of one embodiment of the present invention are taken into consideration, the present invention can also provide the following [I] and [II].
[I] An internal combustion engine, which is installed in a hybrid system, and is filled with the aforementioned lubricating oil composition of one embodiment of the present invention.
[II] A method for lubricating an internal combustion engine, wherein the aforementioned lubricating oil composition of one embodiment of the present invention is applied to an internal combustion engine installed in a hybrid system.

The hybrid system described in the above [I] and [II] is a mechanism having an internal combustion engine and an electromotor as power sources.

Examples of the hybrid system described in the above [I] and [II] include hybrid vehicles, hybrid motorcycles, hybrid trains, and hybrid ships.

The internal combustion engine of the above [I] is filled with the aforementioned lubricating oil composition of one embodiment of the present invention, and is an apparatus installed in a hybrid system together with an electric motor, which is an electromotor.

In addition, the method for lubricating an internal combustion engine of the above [II] specifies the application of the aforementioned lubricating oil composition of one embodiment of the present invention to an internal combustion engine installed in a hybrid system, but the lubricating oil composition may also be applied to an electric motor, which is an electromotor.

As described above, the present invention discloses the following embodiments.
[1] A lubricating oil composition comprising: a base oil (A) comprising an ester base oil (A1); and a hindered amine compound (B),
   wherein a content of the component (B) is 0.60 to 10.0 mass% based on the total amount of the lubricating oil composition.
[2] The lubricating oil composition according to the above [1], wherein a content ratio of the component (A1) is 10 to 100 mass% based on the total amount of the component (A).
[3] The lubricating oil composition according to the above [1] or [2], wherein the component (A1) comprises one or more selected from a polyol ester (A11) and diester (A12).
[4] The lubricating oil composition according to any one of the above [1] to [3], wherein the component (A) comprises an ester base oil (A1) and optionally a mineral oil (A2),
   wherein a content ratio of the mineral oil (A2) is 90 mass% or less based on the total amount of the component (A).
[5] The lubricating oil composition according to any one of the above [1] to [3], wherein the component (A) comprises an ester base oil (A1) and optionally a mineral oil (A2),
   wherein a content ratio of the mineral oil (A2) is 40 mass% or less based on the total amount of the component (A).
[6] The lubricating oil composition according to the above [4] or [5], wherein the component (A) comprises an ester base oil (A1) and a mineral oil (A2).
[7] The lubricating oil composition according to any one of the above [1] to [6], wherein the content of the component (B) based on the total 100 parts by mass of the component (A) is 2.5 parts by mass or more and 50.0 parts by mass or less.
[8] The lubricating oil composition according to any one of the above [1] to [7], wherein the content of the component (B) is 2.50 to 10.0 mass% based on the total amount of the lubricating oil composition.
[9] The lubricating oil composition according to any one of the above [1] to [6], further comprising an antioxidant (C) that does not correspond to the component (B) .
[10] The lubricating oil composition according to the above [9], wherein the component (C) comprises one or more selected from an amine antioxidant (C1) other than a hindered amine compound and a phenolic antioxidant (C2).
[11] The lubricating oil composition according to the above [9] or [10], wherein a content of the component (C) based on the total 100 parts by mass of the component (B) is 1.0 part by mass or more and 100 parts by mass or less.
[12] The lubricating oil composition according to any one of the above [1] to [11], wherein a content of a metal-based detergent in terms of metal atoms is less than 50 ppm by mass based on the total amount of the lubricating oil composition.
[13] The lubricating oil composition according to any one of the above [1] to [12], being used for lubrication of an internal combustion engine of a hybrid system.
[14] An internal combustion engine, which is installed in a hybrid system, and is filled with the lubricating oil composition according to any one of the above [1] to [13] .
[15] A method for lubricating an internal combustion engine, wherein the lubricating oil composition according to any one of the above [1] to [13] is applied to an internal combustion engine installed in a hybrid system.

### Examples

Next, the present invention will be described in much more detail with reference to Examples, but the present invention is in no way limited to these Examples. Measuring methods for various properties are as follows.

### (1) Kinematic viscosity, viscosity index

The kinematic viscosity and viscosity index were measured and calculated in accordance with JIS K2283:2000.

### (2) Contents of calcium atoms (Ca)

The contents were measured in accordance with JPI-5S-38-92.

### (3) Content of nitrogen atoms (N)

The content was measured in accordance with JIS K2609:1998.

### (4) Weight-average molecular weight (Mw)

Measurements were made using a gel permeation chromatograph (HPLC Model 1260 manufactured by Agilent) under the following conditions and the values measured in terms of standard polystyrene were used.

### (Measurement conditions)

Column: Two serially connected "Shodex LF404."
Column temperature: 35°C
Developing solvent: Chloroform
Flow rate: 0.3 mL/min

### Examples 1 to 6 and Comparative Examples 1 to 6

A base oil and various additives were added and mixed in amounts shown in Tables 1 to 2, thereby preparing each lubricating oil composition.

Details of each component used in the preparation of the lubricating oil composition are as follows.

### <Component (Al): ester base oil>

"Polyol ester": Polyol ester corresponding to the component (A11), kinematic viscosity at 40°C = 20 mm²/s, kinematic viscosity at 100°C = 4 mm²/s, viscosity index = 139.

"Diester": Diester corresponding to the component (A12), kinematic viscosity at 40°C = 20 mm²/s, kinematic viscosity at 100°C = 3 mm²/s, viscosity index = 153.

### <Base oil other than component (A1)>

"100N mineral oil": Paraffinic mineral oil classified in Group III of the API base oil categories, kinematic viscosity at 40°C = 20 mm²/s, kinematic viscosity at 100°C = 4 mm²/s, viscosity index = 122.

"PAO (4 cst)": Poly-α-olefin, kinematic viscosity at 100°C = 4 mm²/s, viscosity index = 124.

"PAO (6 cst)": Poly-α-olefin, kinematic viscosity at 100°C = 6 mm²/s, viscosity index = 132.

### <Component (B): hindered amine compound>

"Hindered amine compound": 2,2,6,6-Tetramethylpiperidin-4-yl dodecanoate, compound in which R^{b1} = hydrogen atom and R^{b3} = -C₁₁H₂₃ in the aforementioned general formula (b-11), corresponds to the component (B11), nitrogen atom content = 4.13 mass%.

### <Component (C): antioxidant other than the component (B)>

"Amine antioxidant other than the component (B)": Dinonyldiphenylamine, nitrogen atom content = 3.6 mass%. "Phenolic antioxidant (1)": Thiodiethylenebis[3-(3,5-dit-butyl-4-hydroxyphenyl)propionate].

"Phenolic antioxidant (2)": Benzene propanoic acid-3,5-bis(1,1-dimethylethyl)-4-hydroxyalkyl ester.

### <Other additives>

"Additive mixture (1)": Additive mixture containing an organic molybdenum-based friction modifier, a zinc dithiophosphate (ZnDTP) friction modifier, a boron-modified polyimide, a non-boron modified polyimide, glyceryl monooleate, a silicone anti-foaming agent, a pour point depressant (Mw = 70,000), a viscosity index improver (Mw = 400,000), and the like.

"Additive mixture (2)": Additive mixture containing a calcium-based detergent, an organic molybdenum-based friction modifier, a zinc dithiophosphate (ZnDTP) friction modifier, a boron-modified polyimide, a non-boron modified polyimide, glyceryl monooleate, a silicone anti-foaming agent, a pour point depressant (Mw = 70,000), a viscosity index improver (Mw = 400,000), and the like.

Regarding the lubricating oil compositions prepared, the kinematic viscosity, viscosity index, and the content of Ca atoms were measured or calculated, and the following evaluation tests were carried out. The results of them are set forth in Tables 1 and 2.

### (1) Test for evaluating long-drain properties

The prepared lubricating oil compositions were used to perform an ISOT test for 168 hours with the addition of pure water while injecting NOx gas under the following test conditions, and thereby prepared degraded oils.

### <Test conditions>

Testing machine: ISOT TESTER manufactured by Yoshida Kagaku Kikai Co.,Ltd.
Internal volume of test container: 500 mL
Amount of lubricating oil composition used: 300 mL
Amount of NOx gas: 2,000 ppm by volume based on the total amount of supplied gas
Amount of pure water added: 5 vol% based on the total amount of the lubricating oil composition, added every 24 hours
Agitation speed: 800 r/min
Test temperature (cycle): (1) 4 hours at 60°C, (2) 2 hours at 95°C, (3) 12 hours at 120°C, and (4) 6 hours at 60°C was counted as one cycle and repeated.

Pressure differential scanning calorimetry (PDSC) was performed on the above degraded oils at 180°C and 200 psig oxygen (not flow) in accordance with ASTM D6186-88 to measure the oxidation induction time (OIT), which is the time from the start of measurement to autoxidation. It can be said that the longer the oxidation induction time is, the better the long-drain properties of the lubricating oil composition become. In the present Example, the lubricating oil composition was considered to have good long-drain properties when the oxidation induction time was 50 minutes or more.

### (2) Hot tube test

The degraded oils prepared in the test for evaluating long-drain properties of the above (1) were used to perform a hot tube test in accordance with JPI-5S-55-99 at a test temperature of 240°C. The degree of color change of the glass tube after the test was evaluated on a 21-point scale from 0 (black) to 10 (colorless) (merit rating) in 0.5 increments. It can be said that the higher the score is, the better the high temperature detergency of the lubricating oil composition becomes. In the present Example, the lubricating oil composition was considered to have good high temperature detergency when the score was 7.0 or more.

### [Table 1]

**Table 1**

| | | | | Example 1 | Example 2 | Example 3 | Example 4 | Example 5 | Example 6 |
|---|---|---|---|---|---|---|---|---|---|
| Composition of lubricating oil composition | Component (A1) | Polyol ester | mass% | 86.70 | 83.90 | 60.00 | 40.00 | 20.00 | - |
| | | Diester | mass% | - | - | - | - | - | 83.90 |
| | Base oil other than component (A1) | 100N mineral oil | mass% | | | 23.90 | 43.90 | 63.90 | - |
| | | PAO(4cst) | mass% | - | - | - | - | - | - |
| | | PAO(6cst) | mass% | - | - | - | - | - | - |
| | Component (B) | Hindered amine compound | mass% | 2.80 | 5.60 | 5.60 | 5.60 | 5.60 | 5.60 |
| | Component (C) | Amine antioxidant other than component (B) | mass% | 0.30 | 0.30 | 0.30 | 0.30 | 0.30 | 0.30 |
| | | Phenolic antioxidant (1) | mass% | 0.15 | 0.15 | 0.15 | 0.15 | 0.15 | 0.15 |
| | | Phenolic antioxidant (2) | mass% | 0.50 | 0.50 | 0.50 | 0.50 | 0.50 | 0.50 |
| | Other additives | Additive mixture (1) | mass% | 9.55 | 9.55 | 9.55 | 9.55 | 9.55 | 9.55 |
| | | Additive mixture (2) | mass% | - | - | - | - | - | - |
| | Total | | mass% | 100.00 | 100.00 | 100.00 | 100.00 | 100.00 | 100.00 |
| | Content of component (B) based on the total 100 parts by mass of component (A1) | | part by mass | 3.23 | 6.67 | 9.33 | 14.00 | 28.00 | 6.67 |
| | Content of N derived from component (B) | | mass% | 0.12 | 0.23 | 0.23 | 0.23 | 0.23 | 0.23 |
| | Content of N derived from amine antioxidant other than component (B) | | mass% | 0.011 | 0.011 | 0.011 | 0.011 | 0.011 | 0.011 |
| Properties of lubricating oil composition | Kinematic viscosity at 40°C | | mm²/s | 47.43 | 47.46 | 44.30 | 41.67 | 37.35 | 29.69 |
| | Kinematic viscosity at 100°C | | mm²/s | 10.11 | 10.12 | 9.560 | 9.172 | 8.466 | 7.650 |
| | Viscosity index | | - | 208 | 208 | 208 | 211 | 214 | 245 |
| | Content of Ca in lubricating oil composition | | ppm by mass | 2> | 2> | 2> | 2> | 2> | 2> |
| Evaluation points | Test for evaluating long-drain properties OIT of degraded oil | | min | 126 | 170 | 104 | 78 | 67 | 155 |
| | Hot tube test (240°C) Score | | - | 9.5 | 9.5 | 9.0 | 8.5 | 8.0 | 9.5 |

### [Table 2]

**Table 2**

| | | | | Comparative Example 1 | Comparative Example 2 | Comparative Example 3 | Comparative Example 4 | Comparative Example 5 | Comparative Example 6 |
|---|---|---|---|---|---|---|---|---|---|
| Composition of lubricating oil composition | Component (A1) | Polyol ester | mass% | - | - | - | - | - | - |
| | | Diester | mass% | - | - | - | - | - | - |
| | Base oil other than component (A1) | 100N mineral oil | mass% | 87.51 | 81.35 | 78.55 | | | |
| | | PAO(4cst) | mass% | - | - | - | 74.38 | 73.69 | 71.31 |
| | | PAO(6cst) | mass% | - | - | - | 13.13 | 13.01 | 12.59 |
| | Component (B) | Hindered amine compound | mass% | - | 2.80 | 5.60 | - | 2.80 | 5.60 |
| | Component (C) | Amine antioxidant other than component (B) | mass% | 0.30 | 0.30 | 0.30 | 0.30 | 0.30 | 0.30 |
| | | Phenolic antioxidant (1) | mass% | 0.15 | 0.50 | 0.50 | 0.15 | 0.15 | 0.15 |
| | | Phenolic antioxidant (2) | mass% | 0.50 | 5.50 | 5.50 | 0.50 | 0.50 | 0.50 |
| | Other additives | Additive mixture (1) | mass% | - | 9.55 | 9.55 | - | 9.55 | 9.55 |
| | | Additive mixture (2) | mass% | 11.54 | - | - | 11.54 | - | - |
| | Total | | mass% | 100.00 | 100.00 | 100.00 | 100.00 | 100.00 | 100.00 |
| | Content of component (B) based on the total 100 parts by mass of component (A1) | | part by mass | - | - | - | - | - | - |
| | Content of N derived from component (B) | | mass% | - | 0.12 | 0.23 | - | 0.12 | 0.23 |
| | Content of N derived from amine antioxidant other than component (B) | | mass% | 0.011 | 0.011 | 0.011 | 0.011 | 0.011 | 0.011 |
| Properties of lubricating oil composition | Kinematic viscosity at 40°C | | mm²/s | 34.58 | 32.66 | 32.81 | 32.40 | 29.99 | 30.06 |
| | Kinematic viscosity at 100°C | | mm²/s | 7.93 | 7.694 | 7.745 | 7.381 | 7.022 | 7.063 |
| | Viscosity index | | - | 212 | 218 | 219 | 205 | 209 | 210 |
| | Content of Ca in lubricating oil composition | | ppm by mass | 1940 | 2> | 2> | 1950 | 2> | 2> |
| Evaluation points | Test for evaluating long-drain properties OIT of degraded oil | | min | 37 | 70 | 91 | 45 | 65 | 103 |
| | Hot tube test (240°C) Score | | - | 8.0 | 5.5 | 5.5 | 7.5 | 5.0 | 5.0 |

Table 1 indicates that the lubricating oil compositions prepared in Examples 1 to 6 have excellent high temperature detergency, as well as good long-drain properties when there is water contamination, as a result of containing the components (A1) and (B). On the other hand, Table 2 indicates that the lubricating oil compositions prepared in Comparative Examples 1 to 6 were inferior in at least one of the long-drain properties and high temperature detergency as a result of not containing at least one of the components (A1) and (B).

## Claims

1. A lubricating oil composition comprising: a base oil (A) comprising an ester base oil (A1); and a hindered amine compound (B),
wherein a content of the component (B) is 0.60 to 10.0 mass% based on the total amount of the lubricating oil composition.

2. The lubricating oil composition according to claim 1, wherein a content ratio of the component (A1) is 10 to 100 mass% based on the total amount of the component (A).

3. The lubricating oil composition according to claim 1 or 2, wherein the component (A1) comprises one or more selected from a polyol ester (A11) and diester (A12).

4. The lubricating oil composition according to any one of claims 1 to 3, wherein the component (A) comprises an ester base oil (A1) and optionally a mineral oil (A2),
wherein a content ratio of the mineral oil (A2) is 90 mass% or less based on the total amount of the component (A).

5. The lubricating oil composition according to any one of claims 1 to 3, wherein the component (A) comprises an ester base oil (A1) and optionally a mineral oil (A2),
wherein a content ratio of the mineral oil (A2) is 40 mass% or less based on the total amount of the component (A).

6. The lubricating oil composition according to claim 4 or 5, wherein the component (A) comprises an ester base oil (A1) and a mineral oil (A2).

7. The lubricating oil composition according to any one of claims 1 to 6, wherein the content of the component (B) based on the total 100 parts by mass of the component (A) is 2.5 parts by mass or more and 50.0 parts by mass or less.

8. The lubricating oil composition according to any one of claims 1 to 7, wherein the content of the component (B) is 2.50 to 10.0 mass% based on the total amount of the lubricating oil composition.

9. The lubricating oil composition according to any one of claims 1 to 6, further comprising an antioxidant (C) that does not correspond to the component (B).

10. The lubricating oil composition according to claim 9, wherein the component (C) comprises one or more selected from an amine antioxidant (C1) other than a hindered amine compound and a phenolic antioxidant (C2).

11. The lubricating oil composition according to claim 9 or 10, wherein a content of the component (C) based on the total 100 parts by mass of the component (B) is 1.0 part by mass or more and 100 parts by mass or less.

12. The lubricating oil composition according to any one of claims 1 to 11, wherein a content of a metal-based detergent in terms of metal atoms is less than 50 ppm by mass based on the total amount of the lubricating oil composition.

13. The lubricating oil composition according to any one of claims 1 to 12, being used for lubrication of an internal combustion engine of a hybrid system.

14. An internal combustion engine, which is installed in a hybrid system, and is filled with the lubricating oil composition according to any one of claims 1 to 13.

15. A method for lubricating an internal combustion engine, wherein the lubricating oil composition according to any one of claims 1 to 13 is applied to an internal combustion engine installed in a hybrid system.
